

# UNITED STATES PATENT OFFICE.

WILLIAM A. MCADAMS, OF NEW YORK, N. Y.

## ALUMINIUM ALLOY.

SPECIFICATION forming part of Letters Patent No. 611,016, dated September 20, 1898.

Application filed December 7, 1897. Serial No. 661,017. (No specimens.)

*To all whom it may concern:*

Be it known that I, WILLIAM A. MCADAMS, of New York, (Brooklyn,) in the county of Kings and State of New York, have invented 5 a new and useful Improvement in Aluminium Alloys, of which the following is a specification.

This invention is an improvement in compositions for use in casting articles of various kinds, the composition being an alloy of aluminium consisting of the following ingredients and combined in substantially the proportions stated—viz., aluminium, one hundred and eight ounces; copper, twelve ounces; 15 zinc, thirty-six ounces; nickel, one ounce.

The several ingredients of the composition are taken in substantially the proportions hereinabove stated and are combined in the following manner: The nickel is melted, and 20 to the molten nickel is added the copper. This mixture is then added to the molten aluminium, and then the zinc is added. The composition may then be poured into the

molds and permitted to cool and harden for forming articles of various kinds.

The composition has the following characteristics: It is a silvery white in color and has a luster which remains undimmed by long outside exposure. It has very great breaking strength, with a considerable amount of 25 spring and resilience. Furthermore, while in its molten state it flows very easily under pressure into the mold, whereby the article which it forms is provided with very sharp and smooth corners and edges.

What I claim is—

A composition of matter consisting of aluminium, copper, zinc and nickel in substantially the following proportions, viz., aluminium one hundred and eight ounces, copper 30 twelve ounces, zinc thirty-six ounces and nickel one ounce.

WILLIAM A. MCADAMS.

Witnesses:

FREDK. HAYNES,  
EDWARD VIESER.